

Patented Nov. 11, 1924.

1,514,655

# UNITED STATES PATENT OFFICE.

ALBERT L. CLAPP, OF DANVERS, MASSACHUSETTS, ASSIGNOR TO BECKWITH MANUFACTURING COMPANY, OF BOSTON, MASSACHUSETTS, A CORPORATION OF MAINE.

## FIBER BOARD AND PROCESS OF MANUFACTURING THE SAME.

No Drawing.

Application filed June 23, 1920. Serial No. 391,163.

*To all whom it may concern:*

Be it known that I, ALBERT L. CLAPP, a citizen of the United States, residing at Danvers, in the county of Essex and State 5 of Massachusetts, have invented new and useful Improvements in Fiber Board and Processes of Manufacturing the Same, of which the following is a specification.

This invention has for its object to provide 10 a new material which is capable of being formed into a hard horny mass or into sheets of any desired thickness, and a process of making the same.

I have discovered that, if animal matter 15 such, for example, as tanned leather, ground bone or dried fish scraps are digested under heat and pressure with a large proportion of caustic alkali in the presence of cellulose fiber, a solution is formed which permeates 20 the fibers, and which may be subsequently precipitated therein by the employment of a precipitating agent such as a metal salt, and that this material may be molded, or formed into a single web or a composite sheet, and 25 that the product is strong and more or less water-repellent. Thus I may produce a paper of high tensile strength, or a hard inflexible board, by varying the proportions of the components and the process of 30 manipulating the fibrous mass.

For forming a material somewhat like fiber board or leather board, one may proceed as follows:—Into a digester, which may be closed, are introduced, say, 1000 pounds 35 of cotton fibers (e. g., "linters" or cotton waste), and about 300-500 pounds of comminuted tanned leather (or ground bone, or such dried fish scraps as are ordinarily used for fertilizers), and about 15 pounds of 40 caustic soda and enough water to submerge the foregoing ingredients. The digester is closed, steam is injected from time to time until a pressure of about 50 pounds is reached, and the cooking is continued for 45 about four hours more or less. The tannic acid in the leather is neutralized and the leather breaks down into solution, and the solution permeates or impregnates the cotton fibers. The fibers, because of the cooking, 50 are rendered capable of hydrating more rapidly than before. The contents of the digester are now withdrawn, and are placed in a beating engine with added water to permit free circulation, and are subjected to a beating operation for about five hours.

Then I add to and beat into the mass a precipitating agent, e. g., aluminum sulphate, lead acetate or other suitable metal salt. This product is now introduced into a wet cylinder paper machine, and the fibrous 60 mass is formed thereon in superposed convolutions until an encircling composite sheet of the desirable caliper is obtained, whereupon the sheet is slit, flattened, dried, and, if desired, compressed under high pressure. 65 Instead of being formed into a web, the water may be squeezed from the mass, and the latter molded in suitable molds under pressure.

It is quite evident that, instead of using 70 cotton fiber, I may use other cellulosic materials, such as mechanical wood pulp or chemical wood pulp, e. g., sulphite or soda pulp, or the screenings of such pulp. For example, a very strong and tough wrapping 75 paper may be made by digesting, under the conditions herein recited, 1000 parts (by weight) of wood pulp (preferably sulphate pulp), 100 parts of comminuted tanned leather, and 5 to 10 parts of caustic soda, 80 and after precipitating the animal matter with a metallic salt in a beating engine, subsequent to the beating of the pulpy mass, then forming a sheet therefrom by any suitable sheet-forming paper machine. A sheet 85 so formed possesses greater strength than paper of the same caliper formed in the usual manner from sulphate pulp. For the sulphate pulp, referred to in this example, I may substitute rag fiber, or cotton "linters" 90 or waste, or ground wood or soda or sulphite pulp, or their equivalents.

The digestion of the tanned leather (or its equivalent) under high pressure and temperature with a large proportion of caustic 95 soda, results in a solution, which, according to Graham's test, is non-colloidal, and thus is capable of permeating individual fibers. The animal matter, which thus goes into solution, is precipitated into water-insoluble 100 precipitate, in gelatinous form which dries into a hard colloidal mass.

What I claim is:—

1. A process which comprises digesting 105 cellulosic material, animal matter and a caustic alkali with heat and pressure, and then precipitating the animal matter in solution.

2. A process which comprises digesting 110 cellulosic material, animal matter and a

caustic alkali with heat and pressure, and then precipitating the animal matter in solution with a metal salt.

3. A process which comprises digesting cellulosic material, animal matter and a caustic alkali with heat and pressure, beating the digested mass with water, and then precipitating the animal matter in solution with a metal salt.

10 4. A process which comprises digesting cellulosic material, animal matter and a caustic alkali with heat and pressure, beating the digested mass with water, then pre-

cipitating the animal matter in solution with a metal salt, and finally forming the pulpy <sup>15</sup> mass into a sheet of desired thickness.

5. A fibrous material, the fibers and interstices of which contain an insoluble colloidal precipitate, precipitated by a metal salt from that noncolloidal matter derived from the digestion of leather or the like with a caustic alkali.

In testimony whereof I have affixed my signature.

ALBERT L. CLAPP.